

## UNITED STATES PATENT OFFICE

ROBERT SERGESON, OF MASSILLON, OHIO, ASSIGNOR TO CENTRAL ALLOY STEEL CORPORATION, OF MASSILLON, OHIO, A CORPORATION OF NEW YORK

## METHOD OF NITRIDING STEEL ARTICLES

No Drawing.

Application filed March 28, 1929. Serial No. 350,575.

This invention relates in general to the heat treatment of articles made from steel alloys, for the purpose of placing the articles in a condition to receive thereon a hard, 5 tough, coherent case or coating, when the articles are subsequently nitrided, as by means of ammonia gas.

It has been observed in the nitriding of articles made from steel alloys, that when these 10 articles are nitrided in the "as rolled or annealed" condition, that the case or coating which is formed thereon is usually of an inferior character, that is to say, it is characterized by one or more of the following defects:

15 (1) The depth of penetration of the case is not uniform.

(2) The case is brittle and does not properly adhere to the core.

In consequence of these defects, the articles, when dropped or subjected to abnormal stresses in service, frequently break or spall, and such occurrences have retarded the development of the nitriding industry to a greater extent than any other single factor.

25 As a result of a series of experiments, which I have made, I have discovered that practically all of the aforesaid defects may be more or less completely obviated by subjecting the articles, prior to nitriding same, 30 to a suitable heat treatment.

The character of the heat treatment varies to some extent with the analysis of the steel from which the articles are formed, but in all cases, the articles are uniformly heated 35 to a temperature above their upper critical point and quenched in any suitable manner, as in oil or water. The articles are then drawn at a temperature below their lower critical point, and are then nitrided in the usual manner.

40 As a result of the aforesaid heat treatment, the case on the nitrided articles is found to harder, deeper and tougher than the case on articles nitrided without previous heat treatment. The case adheres firmly to the core and the articles are immune in a high degree from failures due to breakage or spalling, when dropped or subjected to abnormal stresses in service.

50 In order to bring out the effects of heat

treatment on the case depth and hardness, alloy steel specimens containing .35% carbon, .50% manganese, 1.60% chromium, .70% aluminum, .25% silicon and .20% molybdenum were nitrided in the "as rolled" and "heat treated" condition. The heat treatment consisted in heating the specimens to a temperature of 1650° F., quenching them in an oil bath, and then drawing them at a temperature of 1200° F. The "as rolled" and "heat treated" specimens were then nitrided at a temperature of 1000° F. for 20 hours.

The comparative results were as follows:

| Condition before nitriding | Average case depth | Average Brinell hardness |    |
|----------------------------|--------------------|--------------------------|----|
| "As rolled" -----          | .010"              | 850                      | 65 |
| "Heat treated" -----       | .913"              | 1015                     | 70 |

I claim:

1. The method of nitriding articles made from steel alloys, which comprises heating the articles to a temperature above their upper critical point, quenching the articles, drawing the articles at a temperature below their lower critical point, and then nitriding the articles, the object of said heat treatment being to increase the depth and hardness of the nitrided case to a degree greater than is obtainable when the articles are nitrided without being thus previously heat treated.

2. The method of nitriding articles made from steel alloys, which comprises heating the articles to a temperature of about 1650° F., quenching the articles, drawing the articles at a temperature of about 1200° F., and then nitriding the articles, the object of said treatment being to increase the depth and hardness of the nitrided case to a degree greater than is obtainable when the articles are nitrided without being thus previously heat treated.

In testimony whereof I affix my signature.

ROBERT SERGESON.

CERTIFICATE OF CORRECTION.

Patent No. 1,748,623.

Granted February 25, 1930, to

ROBERT SERGESON.

It is hereby certified that error appears in the printed specification of the above numbered patent requiring correction as follows: Page 1, line 70, the dimension .913" should read .013"; and that the said Letters Patent should be read with this correction therein that the same may conform to the record of the case in the Patent Office.

Signed and sealed this 15th day of April, A. D. 1930.

(Seal)

M. J. Moore,  
Acting Commissioner of Patents.